

# United States Patent [19]

Tanizaki et al.

[11] 4,332,689  
[45] Jun. 1, 1982

[54] WATER BASE LUBRICANT COMPOSITION

[75] Inventors: Yoshiharu Tanizaki, Yokohama; Shigeyuki Takase, Kawasaki; Kenichiro Minagawa, Yokohama; Kiyomitu Watanabe, Tokyo, all of Japan

[73] Assignee: Nippon Oil and Fats Co., Ltd., Tokyo, Japan

[21] Appl. No.: 136,578

[22] Filed: Apr. 1, 1980

[30] Foreign Application Priority Data

Sep. 28, 1979 [JP] Japan 125017

[51] Int. Cl.<sup>3</sup> C10M 1/06

[52] U.S. Cl. 252/49.3; 72/42; 252/56 R; 252/56 S; 252/79

[58] Field of Search 252/49.3, 56 R, 56 S, 252/79; 72/42

[56]

References Cited

U.S. PATENT DOCUMENTS

|           |        |                  |          |
|-----------|--------|------------------|----------|
| 3,374,171 | 3/1968 | Davis .....      | 252/49.3 |
| 3,390,084 | 6/1968 | Lake .....       | 252/49.3 |
| 3,959,534 | 5/1976 | Park et al. .... | 252/49.3 |
| 3,980,571 | 9/1976 | Marx .....       | 252/49.3 |
| 4,146,488 | 3/1979 | Martin .....     | 252/49.3 |

FOREIGN PATENT DOCUMENTS

|           |        |             |          |
|-----------|--------|-------------|----------|
| 52-899607 | 8/1977 | Japan ..... | 252/56 R |
| 53-935059 | 5/1978 | Japan ..... | 252/56 R |

Primary Examiner—Curtis R. Davis  
Attorney, Agent, or Firm—Blanchard, Flynn, Thiel,  
Boutell & Tanis

[57]

ABSTRACT

A polymer of polyoxyalkylene glycol monoacrylate or polyoxyalkylene glycol monomethacrylate is very useful as a base of lubricants.

5 Claims, No Drawings

## WATER BASE LUBRICANT COMPOSITION

## BACKGROUND OF THE INVENTION

## Field of the Invention

5

This invention relates to water base lubricant compositions and more particularly relates to water base lubricant compositions which are low in foamability and are useful in a water soluble hydraulic fluid, a heat medium and a metal working fluid.

Heretofore, non-aqueous combustible lubricants whose bases are mineral oil or animal and plant oils, have been used for a hydraulic fluid, a heat medium, a metal working fluid and the like.

Recently, water base lubricants have been adopted in place of the non-aqueous combustible lubricants for the purpose of preventing fires which occur due to the leakage thereof and for the reason that when they are used for a metal working fluid, the treated lubricants are easily washed off from the metal surface.

As the water base lubricants, there are used, in general, water soluble compounds of high molecular weight for upgrading the lubricity and for increasing the viscosity thereof.

As the water base lubricants, there are known polyvinyl alcohol, salts of polymethacrylic acid, cellulose derivatives, polyoxyalkylene compounds and the like.

Especially, the polyoxyalkylene compounds have advantages in that they have low pour points for use as a synthetic lubricant, they are splendid in viscosity characteristics, they form a small quantity of sludge and varnish and they do not corrode sealing materials of all kinds such as metals, rubber and the like.

However, the known polyoxyalkylene compounds have disadvantages in that they are bad in oxidation stability at an elevated temperature, are apt to undergo thermal decomposition and are bad in lubricity because of their poor wetting on a metal surface, and they generate a large amount of foam.

## SUMMARY OF THE INVENTION

It is an object of the present invention to provide a water base lubricant composition which is splendid in lubricity and is low in foamability.

It is an another object of the present invention to provide a water base lubricant composition which is splendid for increasing viscosity and which forms low amounts of sludge.

It is a further another object of the invention to provide a water base lubricant composition which is low in corroding metals.

The present invention is based on the knowledge that a polymer of polyoxyalkylene glycol monoacrylate or polyoxyalkylene glycol monomethacrylate is very useful as a base of a lubricant.

A water base lubricant composition of the present invention comprises 4-80 parts by weight of polymers of polyoxyalkylene glycol monoacrylate or polyoxyalkylene glycol monomethacrylate (hereinafter both are collectively called PAGMA) and 20-96 parts by weight of water. If necessary, 0-50 parts by weight of a water soluble organic solvent may be added to the water soluble lubricant of the present invention.

The polymer of PAGMA of the present invention comprises repeating units having the following formula (1) whose number average molecular weight is less than 100,000:

10



wherein R is H or CH<sub>3</sub>, m is an integer of 2-4 and n is an integer of 2-20.

The polymer of the present invention comprising repeating units of the formula (1) is obtained by polymerizing PAGMA which is shown in the formula (II):

15



wherein R is H or CH<sub>3</sub>, m is an integer of 2-4 and n is an integer of 2-20.

AGMA of the formula (1) may be obtained by subjecting hydroxyalkyl monoacrylate or hydroxyalkyl monomethacrylate to an addition polymerization with ethylene oxide, propylene oxide, butylene oxide or tetrahydrofuran according to the processes which are shown in Japanese Pat. Nos. 899607 and 935059.

The homopolymerization of PAGMA for obtaining the polymers of the present invention is carried out at a temperature of 40°-180° C., preferably 60°-150° C., for 0.5-30 hours, preferably 1-20 hours in an organic solvent using a polymerization initiator.

Because the starting material of PAGMA contains an extremely small quantity of di(meth)acrylate compound, which is a byproduct in the production thereof and in the polymerization, the three dimensional combination occurs, whereby the obtained polymer undergoes gelation to cause it to be nonuniform, it is better for obtaining a uniform polymerization solution to employ a transfer agent.

As for the organic solvents, there are mentioned, methanol, ethanol, n-propanol, isopropanol, n-butanol, sec-butanol, ethylene glycol, monoethyl ether, ethylene glycol monobutyl ether, dimethyl formamide, dimethylsulfoxide, acetonitrile, acetone, methyl ethyl ketone and the like. The organic solvent is used in an amount of 10-5000 parts, preferably 50-2000 parts by weight based on 100 parts by weight of PAGMA used.

As for the polymerization initiator, there are shown benzoyl peroxide, methylethyl ketone peroxide, cumene hydroperoxide, di-t-butyl peroxide, iso-butyroyl peroxide, t-butylperoxyoctanate, dicumyl peroxide, azobisisobutyronitrile and the like.

The said polymerization initiators are used in an amount of 0.01-25 parts, preferably 0.05-15 parts by weight based on the PAGMA used.

As the transfer agents which are usable for the polymerization there are mentioned mercaptans such as dodecylmercaptan and octylmercaptan, and disulfides such as bis-(hydroxyethyl)disulfide, bis-(2-ethylhexyl)-disulfide, thioglycolic acid.

The said transfer agents are used in an amount of 0.5-50 parts by weight based on 100 parts by weight of the PAGMA used.

The polymer of the PAGMA is less than 100,000, preferably 1,000-50,000, in number average molecular weight. The polymer of the PAGMA whose number average molecular weight exceeds 100,000, is poor in the solubility in the solvents.

The polymer of PAGMA may dissolve very well into water, alcohols, glycols and other organic solvents. When some of the PAGMA are insoluble in water, they may be made into an aqueous solution thereof using a solvent which is soluble in water.

As for the above mentioned solvents, there are mentioned lower monohydric alcohols such as methanol, ethanol, propanol and the like, glycols such as ethylene glycol, diethylene glycol, propylene glycol, dipropylene glycol and the like, glycol ethers such as ethylene-glycol monomethyl-ether, ethyleneglycol monomethyl-ether, diethyleneglycol monoethyl-ether, ethyleneglycol monobutyl-ether, diethyleneglycol monobutyl-ether, propyleneglycol monomethyl-ether, dipropyleneglycol monomethyl-ether, propyleneglycol monoethyl-ether, dipropyleneglycol monoethyl-ether, propyleneglycol monobutyl-ether, dipropyleneglycol monobutyl-ether and the like, derivatives of polyoxyalkylene glycol such as polyoxyethylene glycol, polyoxypropylene glycol, polyoxyethylenoxypropylene glycol and the like, and organic solvents such as dimethylformamide, dimethylsulfoxide, acetonitrile, acetone, methyl ethyl ketone, tetrahydrofuran and the like.

If necessary, additives such as an antiwear agent, a rust inhibitor, an antioxidant, an antifoaming agent and the like may be mixed with the water series lubricant to upgrade the properties thereof for lubricant purposes.

As for the antiwear agent, there are mentioned sodium-, potassium-, or amine soap of aliphatic or aromatic carboxylic acid, fatty acid ester, fatty acid amide, phosphoric acid ester of phenols, or higher alcohols, and the like.

Illustrative of the rust inhibitors are sodium mercapto benzotriazole, sodium phosphate, potassium phosphate, sodium and potassium salts of phosphoric acid, nitrite, morpholine and the like.

As the antioxidant, hindered phenol compounds, bisphenol compounds, aromatic amines and the like are mentioned. As the antifoaming agents, there are mentioned silicone series compounds.

The polymers of PAGMA are very effective as a lubricant and they are more particularly effective as a base fluid of a water-glycol-system fire resistant hydraulic fluid and a water soluble metalworking fluid. Further, they are very useful as an antistatic agent, a dying assistant, and a spinning oil for chemical fibers such as polyester, nylon, acrylic fiber, rayon, acetate fiber and the like, and natural fibers such as wool, cotton, silk and the like.

They are also suitable for a cosmetic fluid because they also promptly dissolve into a water-alcohol system solvent and they do not change in quality at a broad range of temperature and PH value of a PAGMA solution.

#### PREFERRED EMBODIMENTS OF THE INVENTION

The term "part" and "%" small mean part by weight and % by weight respectively hereinafter.

##### Preparation of polymer of polyoxyethyleneglycol monomethacrylate (called as PEM-1)

Into a reaction vessel which was equipped with a stirrer, a reflux condenser and a thermometer, there was charged 80 parts of isopropanol which was heated to 80° C. 20 parts of polyoxyethyleneglycol methacrylate (product of Nippon Oil and Fats Co., Ltd., Trade Mark: Blemmer PE-350) whose number average molecular

weight was 425 and into which 0.4 part of benzoyl peroxide (BPO), as a catalyst, was dissolved, were dropped into the reaction vessel for 2½ hours, thereby carrying out a polymerization.

5 Further, 0.4 part of BPO which was dissolved into 3.8 parts of methyl ethyl ketone, was added to the contents of the reaction vessel, followed by aging the same for 5 hours. The resulting polymer was cooled to room temperature and was poured into 1500 parts of ethyl ether, thereby forming a mixture.

10 The obtained precipitate in the lower layer were heated at a reduced pressure of 30 mm Hg and at 40° C. for 2.0 hours to remove ethyl ether, whereby 16.6 parts of polymer of purified polyoxyethyleneglycol monomethacrylate (conversion ratio: 83.1% PEM-1), which was recognized by the infrared spectrum, the nuclear magnetic resonance spectrum and the Gel permeation chromatograph thereof.

##### Preparation of polymer of polyoxyethyleneglycol monoacrylate (called as PEAP-2)

15 Into the same reaction vessel was used in the preparation of PEM-1, there was charged 50 parts of isopropanol and 1.5 parts of dodecylmercaptan as a transfer agent. Further, 50 parts of polyoxyethylene glycol monoacrylate whose number average molecular weight was 418 and into which 0.5 part of BPO was dissolved, were dropped into the reaction vessel at 83° C. for one hour, followed by aging the contents of the reaction vessel for 5 hours.

20 The obtained polymer was precipitated by adding 2000 parts of ethyl ether thereto, followed by heating the same at a reduced pressure to remove the ethyl ether remaining therein, whereby 36 parts of polymers of polyoxyethyleneglycol monoacrylate was obtained.

##### Preparation of polymer of polyoxyethylene glycol monomethacrylate (called as PEM-3)

25 According to the same procedures as described in the preparation of PEM-1, 60 parts of isopropanol and 2 parts of thioglycolic acid was charged into the reaction vessel and 40 parts of polyoxyethylene glycol monomethacrylate whose number average molecular weight was 288 and into which 0.5 part of BPO was dissolved, were dropped into the reaction vessel.

30 The resulting mixture was aged for 5 hours. The obtained polymer was precipitated by adding 2000 parts of ethyl ether, followed by eliminating the ethyl ether remaining in the polymer at a reduced pressure, whereby 31 parts of polymer of purified polyoxyethylene glycol monomethacrylate was obtained.  
(conversion ratio: 72.0%).

##### Preparation of polymer of polyoxyethylenepropylene glycol monomethacrylate (called as PEM-4)

35 According to the same procedures as described in the preparation of PEM-1, 20 parts of polyoxyethylene-propylene glycol monomethacrylate whose number molecular weight was 431 and whose mixing ratio of oxyethylene to oxypropylene was 50:50 and wherein 0.5 part of BPO was dissolved, were dropped into 80 parts of secondary butanol for 1½ hours to react, and the resulting reaction product was aged for 5 hours.

40 The obtained polymer was precipitated by adding 1800 parts of ethyl ether, followed by heating the same at a reduced pressure to remove the ethyl ether therefrom, whereby 15.6 parts of polymer of polyoxy-

5 thylenepropylene glycol monomethacrylate was obtained.

Preparation of polymer of polyoxypropylene glycol monomethacrylate (called as PEMP-5)

According to the same procedures as described in the preparation of PEMP-1, 20 parts of polyoxypropylene glycol monomethacrylate (Nippon Oil and Fats Co., Ltd., Trade Mark Blemmer PP-1000) whose number average molecular weight was 371 and wherein 0.4 part of BPO was dissolved, were dropped into 30 parts of isopropanol for one hour to react, and the resulting product was aged for 6 hours. The obtained polymer was precipitated by adding 1200 parts of n-hexane followed by heating the same at a reduced pressure to 15 remove the n-hexane therefrom, whereby 17.6 parts of polymer of polyoxypropylene glycol monomethacrylate were obtained.

The respective polymers obtained in preparations 1-5, were examined about their respective solubilities to ethanol, tetrahydrofuran and water. Further, gel permeation chromatography analysis was applied to the respective tetrahydrofuran solutions, whereby the respective number average molecular weight and weight average molecular weights were obtained.

The obtained results are shown in Table 1.

TABLE 1

| Polymer | Solubility* |                  |       | Average molecular weight |                |
|---------|-------------|------------------|-------|--------------------------|----------------|
|         | Ethanol     | Tetrahydro-furan | Water | Number average           | Weight average |
| PEMP-1  | ○           | ○                | ○     | 23,900                   | 37,100         |
| PEMP-2  | ○           | ○                | ○     | 16,200                   | 24,000         |
| PEMP-3  | ○           | ○                | ○     | 6,100                    | 9,300          |
| PEMP-4  | ○           | ○                | ○     | 24,100                   | 39,400         |
| PEMP-5  | ○           | ○                | △     | 20,700                   | 31,500         |

Note:

\*Solubility is that obtained at room temperature. Mark ○ shows that a sample dissolves into a solvent uniformly. Mark △ shows that a sample dissolves into 30% ethanol aqueous solution but does not dissolve into water.

EXAMPLES 1 AND 8, COMPARATIVE EXAMPLES 1 AND 2

Respective water base lubricant compositions were prepared by mixing respective bases with the balance of the compositions in the mixing ratio set forth in Table 2. The balance of the compositions had the following recipe.

| The balance of the compositions excluding the base |      | Parts by weight |
|----------------------------------------------------|------|-----------------|
| Water (ion exchanged water)                        | 43.8 |                 |
| Ethylene glycol (solvent)                          | 46.1 |                 |
| Oleic acid                                         | 6.9  |                 |
| Morpholine                                         | 1.2  |                 |
| Potassium hydroxide                                | 1.7  |                 |
| Benzotriazole                                      | 0.24 |                 |
| Silicone compound                                  | 0.06 |                 |

5

10

15

20

25

30

35

40

45

50

55

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

610

615

620

625

630

635

640

645

650

655

660

665

670

675

680

685

690

695

700

705

710

715

720

725

730

735

740

745

750

755

760

765

770

775

780

785

790

795

800

805

810

815

820

825

830

835

840

845

850

855

860

865

870

875

880

885

890

895

900

905

910

915

920

925

930

935

940

945

950

955

960

965

970

975

980

985

990

995

1000

1005

1010

1015

1020

1025

1030

1035

1040

1045

1050

1055

1060

1065

1070

1075

1080

1085

1090

1095

1100

1105

1110

1115

1120

1125

1130

1135

1140

1145

1150

1155

1160

1165

1170

1175

1180

1185

1190

1195

1200

1205

1210

1215

1220

1225</p

TABLE 2-continued

| Polymer<br>glycol | Mixing<br>ratio of<br>a base to<br>the balance | Kinetic                      |                           | Pour<br>point<br>(°C.) | Foaming<br>property | Four ball<br>test by Soda<br>method<br>220rpm<br>(kg/cm <sup>2</sup> ) |           | Oil test by<br>Timken method |                    |
|-------------------|------------------------------------------------|------------------------------|---------------------------|------------------------|---------------------|------------------------------------------------------------------------|-----------|------------------------------|--------------------|
|                   |                                                | viscosity<br>40° C.<br>(Cst) | Viscosity<br>index<br>VIE |                        |                     | 0<br>min                                                               | 10<br>min | Maximum<br>load<br>(lbs)     | Unit load<br>(psi) |

TABLE 3

| Polymer                  | Oxidation<br>Stability                      |                | Corrosion to Metal (mm/cm <sup>2</sup> ) |               |                |               |                |               |                |               |
|--------------------------|---------------------------------------------|----------------|------------------------------------------|---------------|----------------|---------------|----------------|---------------|----------------|---------------|
|                          | Cst(40° C.)PH                               | Viscosity      | Alminium                                 |               | Iron           |               | Steel          | Brass         | Solder         | Copper        |
|                          |                                             |                | Before<br>test                           | After<br>test | Before<br>test | After<br>test | Before<br>test | After<br>test | Before<br>test | After<br>test |
| Example 1                | PEMP-1                                      | Before<br>test | 42.0                                     | 10.9          | -0.071         | -0.037        | -0.018         | -0.102        | -0.073         | -0.061        |
|                          |                                             | After<br>test  | 39.1                                     | 7.3           |                |               |                |               |                |               |
| Example 3                | PEMP-2                                      | Before<br>test | 42.1                                     | 10.7          | -0.065         | -0.025        | -0.027         | -0.233        | -0.064         | -0.057        |
|                          |                                             | After<br>test  | 39.1                                     | 7.2           |                |               |                |               |                |               |
| Example 5                | PEMP-3                                      | Before<br>test | 42.2                                     | 11.1          | -0.039         | -0.015        | -0.031         | -0.097        | -0.135         | -0.195        |
|                          |                                             | After<br>test  | 39.5                                     | 7.8           |                |               |                |               |                |               |
| Example 7                | PEMP-4                                      | Before<br>test | 42.3                                     | 11.2          | -0.053         | -0.042        | -0.012         | -0.084        | -0.181         | -0.088        |
|                          |                                             | After<br>test  | 38.4                                     | 6.9           |                |               |                |               |                |               |
| Comparative<br>Example 1 | Poly-<br>oxyethylene<br>propylene<br>glycol | Before<br>test | 42.1                                     | 11.0          | -0.214         | -0.043        | -0.043         | -0.521        | -0.273         | -0.409        |
|                          |                                             | After<br>test  | 37.1                                     | 5.7           |                |               |                |               |                |               |

Test for working fluid properties of water base lubricants were carried out for the water base lubricants of Example 1, 5, 7 and Comparative Example 1, using a Vein pump which was a oil pressure pump of Vickers Co., Ltd. under the following conditions.

|                               |                      |
|-------------------------------|----------------------|
| amount of sample taken:       | 80l                  |
| discharge pressure:           | 70kg/cm <sup>2</sup> |
| rpm of pump:                  | 1200                 |
| entrance temperature of pump: | 55° C.               |
| testing hours:                | 100 hours            |

The obtained results are shown in Table 4.

TABLE 4

| Polymer                  | Metal wear amount<br>of pump (mg)       |       | Conditions of<br>working fluid |                              | 55                 |
|--------------------------|-----------------------------------------|-------|--------------------------------|------------------------------|--------------------|
|                          | Cume-<br>ring                           | Vein  | To-<br>tal                     | Occur-<br>rence<br>of sludge |                    |
| Example 1                | 192.6                                   | 24.8  | 217.4                          | none                         | transparent        |
| Example 5                | 143.6                                   | 11.3  | 154.9                          | none                         | transparent        |
| Example 7                | 146.2                                   | 37.5  | 183.7                          | none                         | transparent        |
| Comparative<br>Example 1 | Polyoxyethylene<br>propylene-<br>glycol | 794.6 | 43.9                           | 838.5                        | a little<br>cloudy |

It was recognized from Table 4 that the water base lubricants of the present invention are superior to the Comparative example as a working fluid for the reason that the former are transparent and cause less metal

wear amount of the pump than the latter and there is no occurrence of sludge in the former.

As described in the foregoing, the water base lubricant of the present invention is superior to the known polyoxyalkylene glycol compounds in increasing the viscosity thereof and in the lubricity and they are low in foam and are fluid at low temperature.

Accordingly, the water base lubricants of the present invention are very effective for use as a water series lubricant, a water-glycol base fire-resistance hydraulic fluid, a metal molding oil, a cutting or grinding oil and a base or additive for a water base quenching oil.

The embodiments of the invention in which an exclusive property or privilege is claimed are defined as follows:

1. A water-based lubricant comprising a solution of from 20 to 96 parts by weight of water and from 4 to 80 parts by weight of polymer having a number average molecular weight of less than 100,000, said polymer consisting essentially of recurring structural units of the formula



wherein R is H or CH<sub>3</sub>, m is an integer of from 2 to 4, and n is an integer of from 2 to 20.

2. A water-based lubricant as claimed in claim 1 in which the number average molecular weight of said polymer is from 1,000 to 50,000.

3. A water-based lubricant as claimed in claim 1 or claim 2, also containing from zero to 50 parts by weight of a water-soluble organic solvent.

4. A water-based lubricant as claimed in claim 3, also containing an effective amount of one or more lubricant additives selected from the group consisting of an an-

tiwear agent, a rust inhibitor, an antioxidant and an antifoaming agent.

5. A water-based lubricant as claimed in claim 3 consisting essentially of water, said polymer and said water-soluble organic solvent.

\* \* \* \* \*

10

15

20

25

30

35

40

45

50

55

60

65

UNITED STATES PATENT AND TRADEMARK OFFICE  
CERTIFICATE OF CORRECTION

PATENT NO. : 4,332,689

DATED : June 1, 1982

INVENTOR(S) : Yoshiharu Tanizaki et al

It is certified that error appears in the above-identified patent and that said Letters Patent is hereby corrected as shown below:

On the title page the name of the second inventor  
should read

-- Sigeyuki Takase --.

Signed and Sealed this  
Fifteenth Day of March 1983

[SEAL]

Attest:

GERALD J. MOSSINGHOFF

Attesting Officer

Commissioner of Patents and Trademarks